

## UNITED STATES PATENT OFFICE.

WILLIAM C. PERRY, OF KANSAS CITY, MISSOURI.

## MOTOR FUEL.

No Drawing.

Application filed February 27, 1922. Serial No. 539,771.

*To all whom it may concern:*

Be it known that I, WILLIAM C. PERRY, a citizen of the United States, residing at Kansas City, in the county of Jackson and State of Missouri, have invented certain new and useful Improvements in Motor Fuel; and I do declare the following to be a full, clear, and exact description of the invention, such as will enable others skilled in the art to which it appertains to make and use the same.

This invention relates to a combustion engine fuel and particularly to means for preventing the so-called "knock" apparent in the engine resulting from use of the present day gasoline.

I have found that by introducing naphthylamin in the gasoline, the "knock" is not present.

20 This, I believe, is due to the fact that the boiling point of the gasoline is lowered, but from whatever cause, there is an appreciable absence of the so-called "knock" in the gasoline when it is treated with naphthylamin.

25 Naphthylamin is not soluble in gasoline but it is soluble in benzol. In preparing the naphthylamin, I combine it with benzol in the proportions of one-to-one or about 50% each. The benzol and naphthylamin can be mixed either in liquid or vapor phase, the resultant product being a permanent solution of naphthylamin and benzol; that is, a solution which will not separate upon standing.

35 A suitable proportion of the solution is added to the gasoline. While naphthylamin is not soluble in gasoline but is soluble in benzol, the solution of benzol and naphthylamin is readily soluble in gasoline so that when the naphthylamin has been first combined with benzol and then the resultant

product combined with gasoline, there is an effective solution which will not separate upon standing.

I prefer to combine the solution and gasoline in the proportions of from four to six per cent of the gasoline used although these proportions may be varied. When so combined, the so-called "knock" is not present.

45 In actual practice I have found the solution materially improves the gasoline, particularly in causing the absence of the so-called "knock" and in some instances there is an appreciable increase in mileage and power of the engine.

50 Benzol alone will reduce the liability of "knocks" in the gasoline but a relatively large proportion of benzol must be employed and since the amount of benzol available is limited, the amount of gasoline which can be treated would necessarily be limited. By combining naphthylamin with benzol to first provide a solution, a relatively small amount of the solution can be used in the gasoline with equally good results. Therefore, a larger amount of gasoline can be treated than is possible when benzol alone is used.

55 What I claim and desire to secure by Letters Patent is:

1. A motor fuel consisting of gasoline and naphthylamin in solution.

2. A motor fuel consisting of naphthylamin, benzol and gasoline.

3. A motor fuel consisting of a one-to-one 75 solution of naphthylamin and benzol combined with gasoline, the amount of gasoline preponderating over the solution of naphthylamin and benzol.

In testimony whereof I affix my signature.

WILLIAM C. PERRY.